

## UNITED STATES PATENT OFFICE.

RAY G. COATES, OF PASADENA, CALIFORNIA, ASSIGNOR TO VALLEY MOULD AND IRON CORPORATION, OF SHARPSVILLE, PENNSYLVANIA, A CORPORATION OF NEW YORK.

## INGOT MOLD AND METHOD OF MAKING SAME.

No Drawing.

Application filed August 17, 1922. Serial No. 582,545.

*To all whom it may concern:*

Be it known that I, RAY G. COATES, a citizen of the United States, residing at Pasadena, in the county of Los Angeles, State of California, have invented certain new and useful Improvements in Ingot Molds and Methods of Making Same, of which the following is a specification.

This invention relates broadly to metallurgy and more specially to ingot molds used for casting steel ingots.

The principal object of my invention is to increase the number of "heats" an ingot mold will stand before it becomes unfit for service.

Another object is to provide an ingot mold having the mold wall portion adjacent the matrix of the mold under tension at normal temperatures.

20 A further object of the present invention is an ingot mold wherein the normal conditions of stress in mold walls is reversed when the mold is filled with molten metal.

25 A still further object of the present invention is to provide an ingot mold wherein the outer portion of the mold walls is chilled metal and the inner portion of the mold walls is non-chilled metal.

Other and further objects of the present invention will in part be obvious and will in part be pointed out hereinafter in the specification following.

Realizing that the present invention may be carried in constructions other than those herein specifically described it is desired that the disclosure shall be understood as illustrative and not in the limiting sense.

When a common annealed ordinary mold, at normal temperature, is filled with fluid steel the inner surfaces of the mold become rapidly heated from the intense heat of the hot metal. This heat is conducted through the mold walls to the outer surfaces and from these surfaces is dissipated by convection and radiation. Since the inner surfaces are more quickly heated by the fluid steel than a parallel zone in the mold walls, these inner portions of the mold walls tend to expand, and since any expansion is resisted by the still cool outer portion of the walls, a heavy stress of compression results on this part first heated. The effort to expand puts a strong tensile stress on the outer portion of the walls which resist this expansion so

that a condition of considerable stress between the inner and outer parts of the walls results. The expansion of the inner portion of the walls is restrained by a tensile stress on the outer portion of the walls and therefore a high compressional stress exists all over the inner portion of the walls. Thus a very heavy tensile stress occurs in the outer portion of the walls at the time the heat reaches the outer surface of the mold. During this time the inner zone of the mold 55 walls has passed from a condition of no stress to one of high compression. These stresses continue to grow until the heat reaches the outer walls and the heat gradient becomes more or less stable. From this time 60 both walls rise in temperature, although not necessarily at parallel rates, until the highest points reached by the inner walls is attained. At normal temperature the walls of the ordinary mold are as nearly neutral as to 65 all internal stresses as ordinary annealing in the sand will accomplish. When the ordinary mold is filled the stresses in the walls are all in one direction from the neutral condition, a compressional stress on the inner 70 walls and tensile stress on the outer walls.

My improved mold is so cast that when the improved mold is at normal temperature the inner zone of the mold walls is in a state of tension, instead of one of neutrality as in the 75 common mold, which tension is resisted by a compressional stress on the outer zone of the mold walls. This condition of stress may be produced by any of the usual controllable methods now practiced in the foundry which 80 results in strained castings. In casting my improved mold the cooling of the outer walls is to be accelerated as regards that of the inner walls. It is most readily effected by casting the inner surface of the mold against 85 a surface of small heat absorbing capacity and the outer walls against one whose heat absorbing capacity is relatively larger. This more rapid cooling of the outer walls is not carried to the extent of a quick chilling of 90 the outer surface of the mold so as to harden it in the commonly accepted sense of "chilled" metal, although this metal may be considered as having been chilled in the 95 sense that the heat has been rapidly absorbed.

The flask part of the mold in which the ingot mold itself is cast should have a heat

absorbing capacity such that the outer wall of the mold will "set" promptly while the inner wall is to be kept hotter by being cast over a dried core, of such construction as to 5 have a small heat absorbing capacity, so as to not "set" the inner wall of the mold so promptly as the outer wall. The difference in setting and cooling rates causes the outer walls to build up somewhat more rapidly 10 than the inner walls, which latter are therefore at a higher temperature so that as the mold cools down a heat gradient runs from the inner surface towards the outer surface of the mold walls. At the final end of cooling 15 the inner portion of the walls having cooled later than the outer portion of the walls from the temperature of "fluidity" and "setting," these inner portions arrive at normal temperature in a state of tension for 20 the reason that the outer portion of the walls had practically ceased to contract while the inner portions of the walls kept on contracting until it reached normal temperature. This differential effect is rendered possible 25 by the great thickness of the walls of ingot molds. These final strains are not to be removed by annealing. When the metal has solidified so that there is no danger of "bleeding" the cooling of the outer portion 30 of the walls may be accelerated by removing the flask from the casting and letting the air carry off the heat at a more rapid rate, with the secondary advantage of releasing the equipment for other work. The inner 35 portion of the wall, however, is to be protected from cooling effects by being kept in contact with the core sand until the mold is cool.

The improved cool mold is thus in a condition of tension throughout the inner portion of its walls, which tension is resisted by a compressional strain on the outer remaining thickness of the walls.

When fluid steel is poured into such a 45 mold the heat travels by conduction through the mold walls towards their outer surface and simultaneously with this conduction the inner walls tend to begin to expand. Since these inner walls are initially under tension 50 this tendency has the effect of reducing the tension. A reduction of tension on the inner walls simultaneously reduces the compressional stress on the outer walls. The continued conduction of heat from the inner 55 towards the outer walls, with its accompanying expansion, finally brings the heat to the outer surface.

In this course of events at some point in the rise of temperature of the inner walls a 60 point is reached where the expansion of the walls neutralizes the initial tension and a corresponding loss of the compressional strain on the outer wall results. At this state the mold is about in the condition of 65 a common annealed mold as it stands at nor-

mal temperature ready for a "heat." There is a very important difference, however, for the common mold is without strains when cold, while my improved mold is without strains when already well heated towards 70 the maximum temperature it will attain. This condition of neutrality is, of course, of brief duration for the temperature of the walls keeps rising and the inner walls develop a compressional stress because of their 75 continued expansion. Simultaneously because of this rising compressional stress on the inner walls, the outer walls develop tensile stresses, and both of these stresses increase until the heat gradient from the inner to the outer walls has become established 80 after which the temperatures continue to rise in both walls, although not necessarily at parallel rates, with a stress condition 85 more or less unvarying.

The condition of the inner walls of the mold has changed from a tensile stress to a condition of neutrality and then to a condition of compression stress. The fluid steel produces a continuous heating effect 90 on the mold walls but a divided stress effect. The range from the neutral condition being a stress each way, tensile and compressional, it results that the maximum stresses each way are smaller than with the common 95 mold in which the inner walls immediately build up a compressive stress from the beginning of the "heat" so that the final maximum strain point reached represents a departure from the neutral point much greater than in the case of my improved mold. Thus in my mold the inner and outer walls experience both tensile and compressive 100 stresses. In the old mold the inner walls suffer compressional stresses while the outer 105 walls receive only tensile stresses from the beginning of a heat.

It is customary to dry the cores used in casting ingot molds and to "skin dry" at least the sand in the flask. This is the most 110 ready means for "setting" and cooling the metal without contractual stresses, so that such molds, after annealing more or less in the "hot pile" are found to give the customary service.

In casting my improved mold the usual dried core built up on a plain or collapsible core bar may be used. Instead of a common flask filled with sand, a metal form of a suitable thickness and internally of a form 115 closely approximating the outer form of the mold may be used and the inside of this form may be coated with slurry, graphite, white-wash, or brush coat of any satisfactory wash that will act as a non-conductor of heat. 120 Any mechanical means of applying this coat may be used. The object of the coating is to prevent too rapid a chilling action of the flask on the outer surface of the mold being cast, yet to still cool the hot metal consider- 125

ably faster on the outer portion of the walls than along the core. The flask may be made in several places, if necessary, in order to release the casting or to facilitate making 5 of the flask, or to arrange special pockets for "lug" molds or "staples" to be applied in a completed form to the flask. When such a flask is used it will be well heated after casting and may then be cooled down to a 10 reasonable temperature in water and still have enough heat left in it to quickly dry any coating that may be applied to its interior. Thus when the cycle of operations has been started no other heat than that furnished from the operations of casting will 15 be necessary in order to dry any coating applied to the flask.

I do not confine myself to a metal flask as above described. Any means known to 20 the founder's art which will effect the differential rates of cooling as herein set forth I contemplate using.

The effect of heat due to the continued use of the mold may gradually eliminate the 25 strains arranged for in the casting operation. In this case a part of the useful life of the mold will have already passed before the above mentioned condition is reached and the mold will then be in the condition, as 30 to internal strains, of a common mold at the beginning of its period of service.

My invention applies to the common form of ingot mold for casting vertical steel ingots but may be applied to other forms of molds 35 when these latter are so shaped that the strains arranged for the inner parts of the walls may be properly resisted by the outer parts.

Having thus described my invention, what 40 I claim is:

1. A cast metallic ingot mold having the inner portion of its walls in a state of tension in all directions in planes parallel with the surface of the matrix of said mold when said 45 mold is at normal temperature.

2. A cast metallic ingot mold whose inner walls are so stressed in tension at normal temperature that the stresses are removed by the introduction of hot metal into said mold.

50 3. An ingot mold whose inner walls are so stressed at normal temperature that said strains are removed and then built as stresses of the opposite character by the introduction of hot metal into said mold.

55 4. An article of manufacture comprising a cast metallic ingot mold wherein the conditions of stress in the metal of the walls of the mold adjacent the inner and outer surfaces thereof is reversed when the mold is filled with molten metal.

60 5. An article of manufacture comprising a metallic ingot mold having zones of metal under tension adjacent the inner portion of the wall when the mold is at normal temperature.

6. An article of manufacture comprising a cast metallic ingot mold having the metal under compression adjacent the outer portion of the wall when the mold is at normal 70 temperature.

7. An article of manufacture comprising a metallic ingot mold having the outer portion of the mold wall chilled and the inner portion of the mold walls non-chilled.

8. An article of manufacture comprising 75 an unannealed metallic ingot mold wherein the tensile and compressive strains existing in the metallic walls of the mold adjacent the inner and outer surfaces thereof are reversed when the mold is filled with molten 80 metal.

9. The method of casting an ingot mold which comprises providing a core of small heat absorbing capacity, surrounding said 85 core with a metallic flask of relatively high heat absorbing capacity, filling the space between said core and said flask with molten metal and permitting it to cool to normal temperature therebetween.

10. The method of casting an ingot mold 90 which comprises providing a core of small heat absorbing capacity, surrounding said core with a flask of relatively high heat absorbing capacity, filling the space between said core and said flask with molten metal 95 and retaining said flask and said core in position until said mold is substantially cooled to normal temperature.

11. The method of casting an ingot mold which comprises providing a sand core of 100 small heat absorbing capacity, surrounding said core with a metallic flask of relatively high heat absorbing capacity, filling the space therebetween with molten metal, retaining said core in position until said mold 105 is cooled and removing said flask when said mold is partially cooled to accelerate the cooling of the outer walls thereof.

12. The method of casting an ingot mold which comprises providing a sand core of 110 small heat absorbing capacity, surrounding said core with a suitable flask, filling the space therebetween with molten metal and accelerating the cooling of the outer walls of the mold by removing the flask whereby 115 the outer wall of the mold is cooled more rapidly than the inner wall thereof and the inner walls are set with tensile stresses at normal temperatures.

13. The method of casting an ingot mold 120 which comprises freezing and cooling the inner walls of the mold at a slow rate and at the same time freezing and cooling the outer walls at a rapid rate, whereby the inner walls of the mold are set with tensile 125 stresses at normal temperatures which decrease in value when the temperature of the mold is increased.